

## UNITED STATES PATENT OFFICE

2,461,933

RHODIUM ALLOY COATINGS AND METHOD  
OF MAKING SAMEPaul T. Smith, Esmond, and Joseph A. Smith,  
Cranston, R. I.No Drawing. Application December 24, 1947,  
Serial No. 793,756

7 Claims. (Cl. 29—194)

1

Our invention relates to improvements in the electrodeposition of alloy coatings upon articles and particularly relates to the electrodeposition of alloy coatings including rhodium. This is a continuation in part application of our abandoned application for Rhodium alloy coating and articles produced thereby, S. N. 409,317 filed September 2, 1941, which is a continuation in part of our abandoned application for Alloy coatings and articles produced thereby, S. N. 112,142, filed November 21, 1936. We have found that if a suitable electrolyte be prepared employing a soluble rhodium salt and a soluble metal salt of the cobalt nickel group and the electroplating takes place in a sufficiently acid bath that an alloy will be plated upon the article having the characteristics of the metal of higher atomic weight therein in this instance rhodium, even if the proportion of said metal by weight to the metal of the nickel cobalt group is reduced to a proportion of substantially 20 of the nickel-cobalt group to 1 of rhodium. Thus a coating is obtained which if rhodium be employed is substantially acid proof and at least acid resistant, one which is tarnish resistant, bright, hard and substantially white, in other words, having in general the characteristics of rhodium and in certain respects insofar as brightness and hardness is concerned being somewhat brighter than the pure rhodium employed itself.

A further feature of our improved method is that it permits the use of electrolytes weaker in rhodium than heretofore thought possible and the plating from said electrolyte with standard electroplating equipment.

Exactly what takes place in this alloy electrodeposition is not fully understood. It is possible that a nickelate and cobaltate might be formed, but it is believed that a double salt including the metal of the nickel or cobalt group as a base and rhodium also as a base is probably formed in the electrolyte which on the actual passage of current through the electrolyte splits off as a double cation comprising a molecule of rhodium and the metal of the nickel or cobalt group to plate on the cathode with a different alloy crystalline structure than is obtained from a direct plating of the rhodium or the metal of the nickel group, said crystal when plated having more nearly the characteristics of the metal of higher atomic

2

weight therein than that of the metal of lower atomic weight therein but which has essentially different and in many respects better characteristics than either.

5 To provide a non-tarnishable article with a flash outer alloy coating of our improved metal, we may if desired in accordance with the teachings of the prior art, preliminarily electrodeposit a wear resistant coating of substantial depth of tarnish resistant substantially white metal such as nickel, cobalt, or an alloy thereof prior to the electrodeposition of our improved alloy coating aforescribed. This permits a substantially flash outer alloy coating, but it is apparent that substantially similar results may be obtained if the intermediate wear resistant coating be omitted and a longer thicker alloy electrodeposit be deposited upon the article in accordance with our invention.

10 20 In carrying out our improved process the following examples are given as typical, but are not attempted to be exclusive. The article may have a tarnishable metal body or outer surface, but usually comprises an outer surface which will readily receive the electrodeposit. The article may be cleaned if desired by an acid bath or otherwise prepared for electrodeposition in any well known manner in the art. As the initial wear resistant coating of tarnish resistant metal over the body we preferably employ a relatively thick electrodeposit of a metal of the nickel cobalt group and a suitable solution for this electrodeposition may be made up as follows:

|    | Per gallon of water:                                                                                                | Ounces |
|----|---------------------------------------------------------------------------------------------------------------------|--------|
|    | Double nickel ammonium sulphate<br>( $\text{NiSO}_4 \cdot (\text{NH}_4)_2\text{SO}_4$ plus 6 $\text{H}_2\text{O}$ ) | 8      |
|    | Nickel sulphate ( $\text{NiSO}_4$ plus 6 $\text{H}_2\text{O}$ )                                                     | 4      |
| 40 | Ammonium chloride ( $\text{NH}_4\text{Cl}$ )                                                                        | 2      |
|    | Boric acid ( $\text{H}_3\text{BO}_3$ )                                                                              | 2      |

45 with a voltage ranging from 2 to 2.5 for a period of approximately five minutes, this will give a wear resistant coating of the desired thickness.

To provide the outer alloy coating a suitable bath may be made up as follows:

50 Per two gallons of water:  
(3.36 ounces (13 grms.) by weight of metal of

cobalt or and nickel in sulphate, chloride or any soluble form);

(.105 ounces (4. grm.) of metal of rhodium in sulphate, chloride or other soluble form.)

The solution is preferably neutralized by the addition of a solution of sodium carbonate or other suitable alkali and sufficient C. P. sulphuric acid or orthophosphoric acid or any other suitable inorganic acid is added to acidify the solution to a low pH value not in excess of 3.5 (preferably around 1.7) and it has been found that 1 ounce C. P. sulphuric acid or 2 ounces of orthophosphoric acid will be sufficient for this purpose. If desired, however, similar amounts by weight of metal of cobalt or nickel sulphate or phosphate or other soluble salt and similar amounts by weight of rhodium sulphate, phosphate or other soluble salt may be added directly to the bath. If commercial cobalt or nickel sulphate be employed approximately 16 ounces per two gallons may be employed, and if commercial rhodium sulphate or phosphate be employed approximately one ounce of three gram metal solution per ounce may be employed per two gallons. If desired, at least 1 ounce of boric acid may be employed as a stabilizer. Thus an electrolyte was formed by this method containing per liter approximately 12.5 grams by weight of metal of cobalt and/or nickel in a solution of a soluble salt thereof and .4 gram by weight of metal of rhodium in the form of a soluble salt thereof per liter may be employed and to bring the pH value not in excess of 3.5 (preferably around 1.7) 4 c. c. of C. P. sulphuric acid were employed. We have found that cobalt, however, is slightly preferable to nickel as it gives a slightly brighter electrodeposit and will tend to brighten the under coating.

In the electrodeposition of articles with this method with a flash coating of our improved alloy, a current of five volts, an amperage of 10 and a temperature of approximately 120° F. with an immersion of thirty seconds has successfully commercially alloy coated many gross of articles.

We have also found that our improved method readily lends itself to a continuous method and that if the electrolyte be prepared as hitherto stated and the pH kept down below 3.5, a true alloy plating of a metal alloy on said article will take place. In the particular electrolytes specifically mentioned as examples the approximate pH value of the electrolyte was actually around 1.7.

#### Example 2

Grams to 1 liter of water

|                                                        |      |     |
|--------------------------------------------------------|------|-----|
| CoSO <sub>4</sub> ·7H <sub>2</sub> O (12.6 gms. metal) | gms. | 60  |
| Na <sub>2</sub> SO <sub>4</sub>                        | do   | 7.5 |
| H <sub>3</sub> BO <sub>3</sub>                         | do   | 7.5 |
| RhSO <sub>4</sub> (.4 gm. metal)                       | cc.  | 4   |
| H <sub>2</sub> SO <sub>4</sub>                         | do   | 2   |

A 3" x 1" brass strip was plated in this bath for 20 minutes with an amperage of 2½ (60 amp./sq. ft.), a voltage of 4¼ at a temperature of 135-150° F.

An analysis of this alloy plate showed that it comprised substantially 88.4% Co-11.6% Rh.

It will be noted that this is substantially the same formula employed in the example previously given, used commercially in the manufacture of larger units.

#### Example 3

Grams to 1 liter of water

|                                                        |      |     |
|--------------------------------------------------------|------|-----|
| CoSO <sub>4</sub> ·7H <sub>2</sub> O (12.6 gms. metal) | gms. | 60  |
| Na <sub>2</sub> SO <sub>4</sub>                        | do   | 7.5 |
| H <sub>3</sub> BO <sub>3</sub>                         | do   | 7.5 |
| RhSO <sub>4</sub> (.4 gm. metal)                       | cc.  | 4   |
| H <sub>2</sub> SO <sub>4</sub>                         | do   | 2   |

A 3" x 1" brass strip was plated in this bath for 20 minutes with an amperage of 4 (96 amp./sq. ft.), a voltage of 5½, at a temperature of 135-150° F.

An analysis of this alloy plate showed that it contained—

98.3% Co-1.7% Rh

#### Example 4

Grams to 1 liter of water

|                                                        |      |     |
|--------------------------------------------------------|------|-----|
| CoSO <sub>4</sub> ·7H <sub>2</sub> O (12.6 gms. metal) | gms. | 60  |
| Na <sub>2</sub> SO <sub>4</sub>                        | do   | 7.5 |
| H <sub>3</sub> BO <sub>3</sub>                         | do   | 7.5 |
| RhSO <sub>4</sub> (.4 gm. metal)                       | cc.  | 4   |
| H <sub>2</sub> SO <sub>4</sub>                         | do   | 2   |

A 3" x 1" brass strip was plated in this bath for 20 minutes with an amperage of 3½ (84 amp./sq. ft.), a voltage of 5½, at a temperature of 135-150° F.

An analysis of this alloy plate showed that it contained—

95.4% Co-4.6% Rh

#### Example 5

Grams to 1 liter of water

|                                                        |      |     |
|--------------------------------------------------------|------|-----|
| CoSO <sub>4</sub> ·7H <sub>2</sub> O (12.6 gms. metal) | gms. | 60  |
| Na <sub>2</sub> SO <sub>4</sub>                        | do   | 7.5 |
| H <sub>3</sub> BO <sub>3</sub>                         | do   | 7.5 |
| RhSO <sub>4</sub> (.4 gm. metal)                       | cc.  | 4   |
| H <sub>2</sub> SO <sub>4</sub>                         | do   | 2   |

A 3" x 1" brass strip was plated in this bath for 20 minutes with an amperage of 3 (72 amp./sq. ft.), a voltage of 4½, at a temperature of 135-150° F.

An analysis of this alloy plate showed that it contained—

93.1% Co-6.9% Rh

#### Example 6

Grams to 1 liter of water

|                                                         |      |     |
|---------------------------------------------------------|------|-----|
| NiSO <sub>4</sub> ·7H <sub>2</sub> O (13.32 gms. metal) | gms. | 60  |
| Na <sub>2</sub> SO <sub>4</sub>                         | do   | 7.5 |
| H <sub>3</sub> BO <sub>3</sub>                          | do   | 7.5 |
| RhSO <sub>4</sub> (.4 gm. metal)                        | cc.  | 4   |
| H <sub>2</sub> SO <sub>4</sub>                          | do   | 2   |

A 3" x 1" brass strip was plated in this bath for 20 minutes with an amperage of 3 (72 amp./sq. ft.), a voltage of 4½ at a temperature of 135-150° F.

An analysis of this alloy plate showed that it contained—

87% Ni-13% Rh

#### Example 7

Grams to 1 liter of water

|                                                        |      |     |
|--------------------------------------------------------|------|-----|
| CoSO <sub>4</sub> ·7H <sub>2</sub> O (3.15 gms. metal) | gms. | 15  |
| Na <sub>2</sub> SO <sub>4</sub>                        | do   | 7.5 |
| H <sub>3</sub> BO <sub>3</sub>                         | do   | 7.5 |
| RhSO <sub>4</sub> (.4 gm. metal)                       | cc.  | 4   |
| H <sub>2</sub> SO <sub>4</sub>                         | do   | 2   |

A 3" x 1" brass strip was plated in this bath for 20 minutes with an amperage of 2½ (60 amp./sq. ft.), a voltage of 6¼ at a temperature of 135-150° F.

An analysis of this alloy plate showed that it contained—

62% Co-38% Rh

Example 8

Grams to 1 liter of water

|                                                                   |      |     |
|-------------------------------------------------------------------|------|-----|
| Co <sub>2</sub> O <sub>7</sub> H <sub>2</sub> O (5.04 gms. metal) | gms. | 24  |
| H <sub>3</sub> Bo <sub>3</sub>                                    | do   | 7.5 |
| Na <sub>2</sub> SO <sub>4</sub>                                   | do   | 7.5 |
| RhSO <sub>4</sub> (.4 gm. metal)                                  | cc.  | 4   |
| H <sub>2</sub> SO <sub>4</sub>                                    | do   | 2   |

A 3" x 1" brass strip was plated in this bath for 20 minutes with an amperage of 2½ (60 amps./sq. ft.), a voltage of 6, at a temperature of 135-150° F.

An analysis of this alloy plate showed that it contained—

79% Co-21% Rh

Example 9

Grams to 1 liter of water

|                                                                  |      |     |
|------------------------------------------------------------------|------|-----|
| Co <sub>2</sub> O <sub>7</sub> H <sub>2</sub> O (4.2 gms. metal) | gms. | 20  |
| Na <sub>2</sub> SO <sub>4</sub>                                  | do   | 7.5 |
| H <sub>3</sub> Bo <sub>3</sub>                                   | do   | 7.5 |
| RhSO <sub>4</sub> (.4 gm. metal)                                 | cc.  | 4   |
| H <sub>2</sub> SO <sub>4</sub>                                   | do   | 2   |

A 3" x 1" brass strip was plated in this bath for 20 minutes with an amperage of 2½ (60 amp./sq. ft.), a voltage of 5% at a temperature of 135-150° F.

In Examples 2-9 the pH was measured with a quinhydrone and was around 1.7.

An analysis of this alloy plate showed that it contained—

75.2 Co%-24.8% Rh

We have discovered that the cathode current density affects the ratios of metals in the alloys plated from the same bath, thus as shown in Example 2 we employ a cathode current density of 60 amps. per square foot and as shown in Example 3 a cathode current density of 96 amps. per square foot. It will be noted that the greater the cathode current density, the larger relative amount of the metal of the nickel-cobalt group is plated out in the alloy.

As stated, we have found that our improved alloys stand a nitric acid test better than pure rhodium. Thus we plated a flash coat of the alloy given in Example 2 on a nickel base and applied a drop of nitric acid. The nitric acid took approximately 5 minutes to penetrate through. We then applied a flash coat of pure rhodium to a nickel base and applied a drop of nitric acid. This penetrated the flash coat in about thirty seconds, thus tending to prove that our improved alloy is ten times as resistant to nitric acid as the rhodium flash coat employed. As stated above, we believe this is due to the fact that our improved alloy has a much finer crystal than pure rhodium. Our improved alloy may also be employed as a base for a pure rhodium flash coat or thicker electrodeposit to provide a better acid and corrosion proof base for a purer white coat of rhodium.

We have also discovered that if the cathode current density becomes less than 40 amps. per square foot, pure rhodium only will be plated out. We have also discovered that if the pH is allowed to drop below one, that even with a high cathode current density pure rhodium only will be plated out. The pH's given apply in general to the temperatures given varying between 120° and 150° F.

Any insoluble anodes may be used such as

platinum, lead, etc., or anodes alloyed in the same proportions as the metals in the bath.

Employing our improved process, articles have been continuously produced at a much less cost than articles finished with a flash outer electrodeposit of rhodium having in certain respects qualities having more appeal to the trade. The pH's referred to herein have been measured by a quinhydrone electrode.

It is understood that our invention is not limited to the specific embodiments shown or methods described and that various deviations may be made therefrom without departing from the spirit and scope of the appended claims.

What we claim is:

1. The method of alloy plating a metal article with an alloy having the characteristics of the metal of higher atomic weight therein, comprising, immersing said article in an aqueous solution containing a soluble metal salt of the group consisting of nickel and cobalt and a soluble rhodium salt in amounts varying from 3.55 to 13.72 grams of total dissolved metal per liter by weight of metal in proportions by weight of nickel or cobalt to rhodium varying from 8 to 1 to 33.3 to 1 and free inorganic acid, adjusting the pH value of said bath by the addition of free inorganic acid to a value not less than 1 and not in excess of around 1.7 and passing current through said bath with a cathode current density from about 40 to about 96 amperes per square foot and at a temperature from about 120° F. to about 150° F. to cause alloy plating of a metal alloy on said article with an alloy plate containing from 62-38 to 98.3-1.7% by weight of the respective metals.

2. An article having a tarnishable metal body, a wear resistant coating of tarnish resistant substantially white metal of at least one of the group consisting of nickel and cobalt over the body and an acid resistant, tarnish resistant, bright, hard, substantially white electrodeposited outer alloy coating consisting essentially of 95.4-98.3% by weight of metal of at least one of the group consisting of nickel and cobalt and 4.6-1.7% by weight of rhodium having characteristics of the metal of higher atomic weight, namely rhodium, therein.

3. An article having a metal body and a substantially acid-proof bright, hard, substantially white electrodeposited outer alloy coating consisting essentially of 95.4-98.3% by weight of metal of at least one of the group consisting of nickel and cobalt and 4.6-1.7% by weight, of rhodium, having characteristics of the metal of higher atomic weight, namely rhodium, therein.

4. An article having a tarnishable metal body, a wear resistant coating of tarnish resistant substantially white metal of at least one of the group consisting of nickel and cobalt over the body and an acid resistant, tarnish resistant, bright, hard, substantially white electrodeposited outer alloy coating consisting essentially of 75.2-98.3% of one of the group consisting of nickel and cobalt and 24.8-1.7% of rhodium, having characteristics of the metal of higher atomic weight, namely rhodium, therein.

5. An article having a tarnishable metal body, a wear resistant coating of tarnish resistant substantially white metal of at least one of the group consisting of nickel and cobalt over the body and an acid resistant, tarnish resistant, bright, hard, substantially white electrodeposited outer alloy coating consisting essentially of 62-98.3% of one of the group consisting of

nickel and cobalt and 38-1.7% of rhodium, having characteristics of the metal of higher atomic weight, namely rhodium, therein.

6. An article having a tarnishable metal body, and an acid resistant, tarnish resistant, bright, 5 hard, substantially white electrodeposited outer alloy coating consisting essentially of 75.2-98.3% of one of the group consisting of nickel and cobalt and 24.8-1.7% of rhodium, having characteristics of the metal of higher atomic 10 weight, namely rhodium, therein.

7. An article having a tarnishable metal body, and an acid resistant, tarnish resistant, bright, hard, substantially white electrodeposited outer alloy coating consisting essentially of at least 15 62-98.3% of one of the group consisting of nickel and cobalt and 38-1.7% of rhodium, having characteristics of the metal of higher atomic weight, namely rhodium, therein.

PAUL T. SMITH. 20  
JOSEPH A. SMITH.

## REFERENCES CITED

The following references are of record in the file of this patent:

## UNITED STATES PATENTS

| Number    | Name        | Date          |
|-----------|-------------|---------------|
| 543,824   | Altman      | July 30, 1895 |
| 1,029,152 | Tebbetts    | June 11, 1912 |
| 1,717,468 | Schulte     | June 18, 1929 |
| 1,947,180 | Bart        | Feb. 13, 1934 |
| 1,970,950 | Wise        | Aug. 31, 1934 |
| 2,303,497 | Reeve       | Dec. 1, 1942  |
| 2,354,409 | Strasser    | July 25, 1944 |
| 2,432,894 | Holt et al. | Dec. 16, 1947 |